

# United States Patent Office

3,102,832

Patented Sept. 3, 1963

1

3,102,832

## MAGNETIC SHEETS OF LOW ALUMINUM-IRON ALLOYS

Paul A. Albert, Pittsburgh, Pa., assignor to Westinghouse Electric Corporation, East Pittsburgh, Pa., a corporation of Pennsylvania  
No Drawing. Filed Apr. 30, 1958, Ser. No. 731,860  
5 Claims. (Cl. 148—120)

This invention relates to magnetic aluminum-iron alloy materials that exhibit both a high magnetic saturation and a large amount of double orientation, and therefore a high permeability.

It is an object of the present invention to provide aluminum-iron alloys, and shapes thereof, that are characterized by a high amount of cube-on-face grain orientation and a high magnetic saturation.

It is a further object of the present invention to provide a magnetic aluminum-iron alloy according to the foregoing object in which no deleterious alpha-gamma transformation occurs during or subsequent to heat treatment of the alloy.

These objects are attained in accordance with my discoveries in aluminum-iron alloys with low aluminum content. Sheets of alloys are prepared for use in magnetic applications by a rolling and annealing schedule which, in conjunction with the particular compositions involved, characterize the resulting products with a high magnetic saturation and a large amount of double orientation, and thus a high permeability. Consequently, outstanding magnetic materials can be prepared in accordance with my discoveries that have particular utility for such applications as in rotating machinery, because maximum flux level can be experienced without incurring disproportionate copper losses in these magnetic materials. It is also apparent that these materials are further desirable as an aid to minimizing the copper required in a winding in a rotating device since the material has a high permeability.

The materials used in practicing the present invention are aluminum-iron alloys in which the aluminum content is minimized but yet is sufficient to suppress the alpha-gamma transformation evidenced in substantially pure iron upon heat treatment. To secure the highest saturation value, the aluminum content should be kept as small as possible. However, sufficient aluminum must be present to suppress the alpha-gamma transformation and permit retention of the orientation characteristics obtained in the rolling-annealing schedule hereinafter described. Accordingly, the aluminum content should be in an amount sufficient to suppress the alpha-gamma transformation in the resulting alloy but not more than a maximum of about 1.5 percent by weight. While on a theoretical basis it can be said that the amount of aluminum should be minimized so that the highest saturation can be obtained, for practical considerations of commercial practice slightly more than a minimum amount is generally used. Hence the practical minimum is on the order of one percent by weight of aluminum.

Alloys for use in practicing my invention can readily be prepared in accordance with conventional techniques. A satisfactory procedure involves melting electrolytic iron of a purity of at least about 99 percent and then adding commercially pure aluminum of a purity of at least about 99.9 percent to the melt. The melt may be prepared in a vacuum furnace under a partial pressure, e.g. on the order of about one-half atmosphere, of helium or other protective gas. The melt normally is poured under the protective atmosphere to minimize aluminum loss. I have found it convenient to pour at the melting pressure. The solidified alloy then is hot rolled, i.e. at a temperature on the order of 800° to 1000° C. or more, to prepare a plate of the alloy for subsequent rolling and an-

2

nealing in accordance with the invention. Generally the ingot is hot rolled to a plate of a thickness on the order of about 0.40 to 0.75 inch, for this has been found to be a convenient starting point for the subsequent cold rolling operations.

The plate of aluminum-iron prepared as just described is then cold rolled to the final thickness, i.e. to a thickness on the order of 2 to 30 mils or more. As pointed out above, the resulting products are of particular use in rotating machinery. For this reason, the thicker gauges of about 20 to 30 mils are preferred. Aluminum-iron with about 1 to 1.5 percent of aluminum is ductile and may be cold rolled at room temperature. If desired, warm rolling, i.e. at a temperature up to about 650° C., can be used. When the final thickness is obtained, the sheet is annealed.

To obtain the most desirable characteristics in the final product, a particular annealing schedule is followed. In accordance with my discoveries this involves subjecting the alloy sheet to a temperature of about 650° to 800° C. in dry hydrogen or other protective gas for about 1/2 to 2 hours or more. The strip suitably is then furnace cooled, or cooled in a cooling chamber, to a temperature below about 400° C. to about room temperature. Thereafter the cooled material is placed in a furnace at a temperature of about 950° to 1250° C. in an atmosphere of dry hydrogen or other protective gas, and the sheet is annealed at this temperature for at least about one hour and generally for about 2 to 4 hours. Products with good characteristics may also be obtained with a single annealing step. In this latter procedure, just the high temperature, or final, anneal is used. Similarly where a double annealing schedule is used, good properties can be developed even upon omitting the cooling step between the anneals.

In the foregoing manner, strips, sheets and other shapes of the alloys described are produced having a high degree of cube-on-face, or double, orientation. Generally the products are characterized by at least 50% of the grains having cube-on-face orientation. It is evident, therefore, that the materials produced will be characterized, magnetically, with properties more nearly approaching those of single crystals than commercial magnetic materials used for these general purposes.

The invention will be described further in conjunction with the following example. It should be understood that the details are given by way of illustration and are not to be construed as limiting on the invention.

Electrolytic flake iron of a purity of 99.9% was placed in a magnesia crucible in a vacuum furnace provided with a resistance winding. The furnace was evacuated and then repressured to about one-half atmosphere with helium. The iron was then melted. Commercially pure aluminum (purity 99.99%) was added to the melt from within the furnace. When the melt was deemed to be uniform, it was poured into a ingot mold within the furnace and then permitted to solidify.

When the ingot had cooled, it was reheated to about 950° C. and then hot rolled to a thickness of 0.50 inch. The resulting plate was permitted to cool to room temperature whereupon it was cold rolled at about room temperature to a sheet of a thickness of 0.025 inch.

The sheet thereby obtained was placed in an annealing furnace containing an atmosphere of dry hydrogen and maintained there at a temperature of 700° C. for about one hour. At the end of this period the sheet was placed in a cooling chamber and permitted to cool to about room temperature. Then the sheet was placed in a furnace containing an atmosphere of dry hydrogen at 1200° C. and held for two hours. At the end of this time it was air cooled.

Strips of material produced as just described were sub-

jected to routine D.-C. testing procedures to determine the magnetic properties. The data obtained are as follows:

TABLE I

| Iron alloy | Alloy element | $\mu_{max.}$ | $H_s$ | $B_1^*$ | $B_{10}^*$ | $B_{100}^*$ | $B_{1000}^*$ | $H(B=10)$ | $B_s$ |
|------------|---------------|--------------|-------|---------|------------|-------------|--------------|-----------|-------|
| Si-Fe      | 2.65% Si      | 8,600        | .58   | 8.0     | 14.5       | 17.4        | 7.9          | 3.2       | 20.4  |
| Si-Fe      | 1.30% Si      | 6,800        | .85   | 5.3     | 13.8       | 17.3        | 8.7          | 2.11      | 21.1  |
| Si-Fe      | .70% Si       | 6,000        | .94   | 4.5     | 14.0       | 17.5        | 8.2          | 2.52      | 21.2  |
| Si-Fe      | .25% Si       | 2,000        | 2.0   | 1       | 14.0       | 17.9        | 8.5          | 4.0       | 21.4  |
| Al-Fe      | 1% Al         | 14,000       | .31   | 12.0    | 16.7       | 19.0        | -----        | 0.70      | 21.2  |

<sup>1</sup> In kilogausses, averaged in the rolling and transverse directions in the sheet.

Each of the silicon-iron alloys tested in Table I was a commercial product and the data tabularized are the published data on these materials. The aluminum-iron was prepared in accordance with this invention. From these data, it will be noted that in the first two silicon-irons the saturation induction is high but the maximum permeability is only a moderate value. It is believed that those alloys were not subject to alpha-gamma transformation. In the alloy containing 0.25 silicon it will be noted that a very high saturation induction was obtained. However, in that case the maximum permeability was seriously degraded, probably due to the occurrence of transformation. The aluminum-iron, on the other hand, evidenced a saturation induction on the order of the best of the silicon-irons and had a maximum permeability far superior to any of the other alloys. While this is the most outstanding characteristic developed in the materials, it may be noted from the remaining data that significant improvement was obtained in each of the properties tested for which values are given in Table I. About 60% of the grains were double oriented.

A series of tests were conducted on sheets of two commercial silicon-irons and an alloy prepared in accordance with this invention to determine comparative loss data. The results obtained are as follows:

TABLE II  
60 Cycle Loss Data for 1% Al-Fe vs. Other  
Materials at Indicated Kilogausses

| Material    | Core losses (watts/#),<br>$p_o$ |        |        | Exciting volt-amperes,<br>$p_a$ |        |        | A.-C. permeability, $\mu$ |        |        |
|-------------|---------------------------------|--------|--------|---------------------------------|--------|--------|---------------------------|--------|--------|
|             | 10/kg.                          | 15/kg. | 17/kg. | 10/kg.                          | 15/kg. | 17/kg. | 10/kg.                    | 15/kg. | 17/kg. |
| 1.1% Al-Fe  | 1.16                            | 2.80   | 3.90   | 1.47                            | 3.73   | 8.35   | 6,850                     | 5,790  | 1,800  |
| 0.25% Si-Fe | 2.5                             | 5.4    | 7.5    | 11.1                            | 19.4   | 55.5   | -----                     | 1,820  | 670    |
| 2.65% Si-Fe | 1.2                             | 2.8    | 3.3    | 18.0                            | 45.0   | 90.0   | -----                     | 2,150  | -----  |

From these data in Table II it can be concluded that the advantages of increased maximum permeability, both A.-C. and D.-C., and the high magnetic saturation induction that characterize products obtained in accordance with my invention are not secured at a sacrifice in other properties such, for example, as core losses. The aluminum-iron shows a core loss comparable to or improved over that for the silicon-irons. Moreover the exciting volt amperes for these magnetic products is vastly improved over that of silicon-irons.

From the foregoing disclosure and data, it is evident that my invention provides magnetic materials with properties that make them highly useful for a wide variety of magnetic applications.

In accordance with the provisions of the patent statute, the principle of the invention has been explained and there is described what is considered to represent its best embodiment. However, it is to be understood that the invention may be practiced otherwise than as specifically described.

I claim as my invention:

1. A method of producing magnetic sheet characterized

by a high maximum permeability, a high magnetic saturation induction and at least 50 percent of its grains having a cube-on-face orientation which comprises cold rolling without any intermediate annealing a hot-rolled aluminum-iron alloy plate of a thickness of about 0.40 to 0.75 inch, which alloy consists essentially of aluminum in an amount sufficient to prevent alpha-gamma transformation, the aluminum being present in an amount of from about 1 percent but not in excess of about 1.5 weight percent and the remainder iron, to a sheet of a thickness of 2 to 30 mils, annealing the resulting sheet in a protective atmosphere at a temperature of about 650° to 800° C., and then further annealing the sheet in a protective atmosphere at a temperature of about 950° to 1250° C.

2. A method in accordance with claim 1 in which said alloy is slowly cooled to about room temperature between said annealing steps.

3. A method in accordance with claim 1 in which said alloy is cold rolled to a thickness of about 20 to 30 mils.

4. A method in accordance with claim 2 in which said first annealing step is extended for about 1 to 2 hours and said second annealing step is extended for at least 40 1½ hours.

5. A method of producing magnetic materials characterized by high maximum permeability, a high magnetic saturation induction and at least 50 percent of the grains having cube-on-face orientation which comprises cold rolling without any intermediate annealing a hot-rolled aluminum-iron alloy plate of a thickness of about 0.4 to 0.75 inch, which alloy consists essentially of aluminum in an amount of from about 1 to 1.5 weight percent and the remainder iron, to a thickness of about 20 to 30 mils, annealing the resulting sheet in dry hydrogen at a temperature of about 650° to 800° C. for ½ to 2 hours, slowly cooling the annealed sheet, and then further annealing the sheet in an atmosphere of dry hydrogen at a temperature of about 1150° to 1250° C. for about 1 to 4 hours.

70  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
560  
561  
562  
563  
564  
565  
566  
567  
568  
569  
570  
571  
572  
573  
574  
575  
576  
577  
578  
579  
580  
581  
582  
583  
584  
585  
586  
587  
588  
589  
590  
591  
592  
593  
594  
595  
596  
597  
598  
599  
600  
601  
602  
603  
604  
605  
606  
607  
608  
609  
610  
611  
612  
613  
614  
615  
616  
617  
618  
619  
620  
621  
622  
623  
624  
625  
626  
627  
628  
629  
630  
631  
632  
633  
634  
635  
636  
637  
638  
639  
640  
641  
642  
643  
644  
645  
646  
647  
648  
649  
650  
651  
652  
653  
654  
655  
656  
657  
658  
659  
660  
661  
662  
663  
664  
665  
666  
667  
668  
669  
670  
671  
672  
673  
674  
675  
676  
677  
678  
679  
680  
681  
682  
683  
684  
685  
686  
687  
688  
689  
690  
691  
692  
693  
694  
695  
696  
697  
698  
699  
700  
701  
702  
703  
704  
705  
706  
707  
708  
709  
710  
711  
712  
713  
714  
715  
716  
717  
718  
719  
720  
721  
722  
723  
724  
725  
726  
727  
728  
729  
730  
731  
732  
733  
734  
735  
736  
737  
738  
739  
740  
741  
742  
743  
744  
745  
746  
747  
748  
749  
750  
751  
752  
753  
754  
755  
756  
757  
758  
759  
760  
761  
762  
763  
764  
765  
766  
767  
768  
769  
770  
771  
772  
773  
774  
775  
776  
777  
778  
779  
780  
781  
782  
783  
784  
785  
786  
787  
788  
789  
790  
791  
792  
793  
794  
795  
796  
797  
798  
799  
800  
801  
802  
803  
804  
805  
806  
807  
808  
809  
810  
811  
812  
813  
814  
815  
816  
817  
818  
819  
820  
821  
822  
823  
824  
825  
826  
827  
828  
829  
830  
831  
832  
833  
834  
835  
836  
837  
838  
839  
840  
841  
842  
843  
844  
845  
846  
847  
848  
849  
850  
851  
852  
853  
854  
855  
856  
857  
858  
859  
860  
861  
862  
863  
864  
865  
866  
867  
868  
869  
870  
871  
872  
873  
874  
875  
876  
877  
878  
879  
880  
881  
882  
883  
884  
885  
886  
887  
888  
889  
890  
891  
892  
893  
894  
895  
896  
897  
898  
899  
900  
901  
902  
903  
904  
905  
906  
907  
908  
909  
910  
911  
912  
913  
914  
915  
916  
917  
918  
919  
920  
921  
922  
923  
924  
925  
926  
927  
928  
929  
930  
931  
932  
933  
934  
935  
936  
937  
938  
939  
940  
941  
942  
943  
944  
945  
946  
947  
948  
949  
950  
951  
952  
953  
954  
955  
956  
957  
958  
959  
960  
961  
962  
963  
964  
965  
966  
967  
968  
969  
970  
971  
972  
973  
974  
975  
976  
977  
978  
979  
980  
981  
982  
983  
984  
985  
986  
987  
988  
989  
990  
991  
992  
993  
994  
995  
996  
997  
998  
999  
1000  
1001  
1002  
1003  
1004  
1005  
1006  
1007  
1008  
1009  
10010  
10011  
10012  
10013  
10014  
10015  
10016  
10017  
10018  
10019  
10020  
10021  
10022  
10023  
10024  
10025  
10026  
10027  
10028  
10029  
10030  
10031  
10032  
10033  
10034  
10035  
10036  
10037  
10038  
10039  
10040  
10041  
10042  
10043  
10044  
10045  
10046  
10047  
10048  
10049  
10050  
10051  
10052  
10053  
10054  
10055  
10056  
10057  
10058  
10059  
10060  
10061  
10062  
10063  
10064  
10065  
10066  
10067  
10068  
10069  
10070  
10071  
10072  
10073  
10074  
10075  
10076  
10077  
10078  
10079  
10080  
10081  
10082  
10083  
10084  
10085  
10086  
10087  
10088  
10089  
10090  
10091  
10092  
10093  
10094  
10095  
10096  
10097  
10098  
10099  
100100  
100101  
100102  
100103  
100104  
100105  
100106  
100107  
100108  
100109  
100110  
100111  
100112  
100113  
100114  
100115  
100116  
100117  
100118  
100119  
100120  
100121  
100122  
100123  
100124  
100125  
100126  
100127  
100128  
100129  
100130  
100131  
100132  
100133  
100134  
100135  
100136  
100137  
100138  
100139  
100140  
100141  
100142  
100143  
100144  
100145  
100146  
100147  
100148  
100149  
100150  
100151  
100152  
100153  
100154  
100155  
100156  
100157  
100158  
100159  
100160  
100161  
100162  
100163  
100164  
100165  
100166  
100167  
100168  
100169  
100170  
100171  
100172  
100173  
100174  
100175  
100176  
100177  
100178  
100179  
100180  
100181  
100182  
100183  
100184  
100185  
100186  
100187  
100188  
100189  
100190  
100191  
100192  
100193  
100194  
100195  
100196  
100197  
100198  
100199  
100200  
100201  
100202  
100203  
100204  
100205  
100206  
100207  
100208  
100209  
100210  
100211  
100212  
100213  
100214  
100215  
100216  
100217  
100218  
100219  
100220  
100221  
100222  
100223  
100224  
100225  
100226  
100227  
100228  
100229  
100230  
100231  
100232  
100233  
100234  
100235  
100236  
100237  
100238  
100239  
100240  
100241  
100242  
100243  
100244  
100245  
100246  
100247  
100248  
100249  
100250  
100251  
100252  
100253  
100254  
100255  
100256  
100257  
100258  
100259  
100260  
100261  
100262  
100263  
100264  
100265  
100266  
100267  
100268  
100269  
100270  
100271  
100272  
100273  
100274  
100275  
100276  
100277  
100278  
100279  
100280  
100281  
100282  
100283  
100284  
100285  
100286  
100287  
100288  
100289  
100290  
100291  
100292  
100293  
100294  
100295  
100296  
100297  
100298  
100299  
100300  
100301  
100302  
100303  
100304  
100305  
100306  
100307  
100308  
100309  
100310  
100311  
100312  
100313  
100314  
100315  
100316  
100317  
100318  
100319  
100320  
100321  
100322  
100323  
100324  
100325  
100326  
100327  
100328  
100329  
100330  
100331  
100332  
100333  
100334  
100335  
100336  
100337  
100338  
100339  
100340  
100341  
100342  
100343  
100344  
100345  
100346  
100347  
100348  
100349  
100350  
100351  
100352  
100353  
100354  
100355  
100356  
100357  
100358  
100359  
100360  
100361  
100362  
100363  
100364  
100365  
100366  
100367  
100368  
100369  
100370  
100371  
100372  
100373  
100374  
100375  
100376  
100377  
100378  
100379  
100380  
100381  
100382  
100383  
100384  
100385  
100386  
100387  
100388  
100389  
100390  
100391  
100392  
100393  
100394  
100395  
100396  
100397  
100398  
100399  
100400  
100401  
100402  
100403  
100404  
100405  
100406  
100407  
100408  
100409  
100410  
100411  
100412  
100413  
100414  
100415  
100416  
100417  
100418  
100419  
100420  
100421  
100422

## UNITED STATES PATENTS

|           |                       |               |
|-----------|-----------------------|---------------|
| 2,300,336 | Bozorth et al. -----  | Oct. 27, 1942 |
| 2,826,520 | Rickett -----         | Mar. 11, 1958 |
| 2,830,922 | Ahles -----           | Apr. 15, 1958 |
| 2,875,114 | Albert -----          | Feb. 24, 1959 |
| 2,940,882 | Hubbard et al. -----  | June 14, 1960 |
| 2,943,007 | Walter et al. -----   | June 28, 1960 |
| 3,058,857 | Pavlovic et al. ----- | Oct. 16, 1962 |

## FOREIGN PATENTS

|                  |                                                         |              |
|------------------|---------------------------------------------------------|--------------|
| 1,009,214        | Germany -----                                           | May 29, 1957 |
| OTHER REFERENCES |                                                         |              |
| 5                | K. J. Sixtus: Physics, vol. 6, pp. 105-111, March 1935. |              |
|                  | "Ferromagnetism," by Bozorth, copyright 1951 by D.      |              |
|                  | Van Nostrand Co., Inc., pp. 210-220.                    |              |